

N. P. BUMP.

GUN STOCK FOR RIFLES, GUNS, AND SMALL ARMS.

APPLICATION FILED MAY 29, 1918.

1,376,917.

Patented May 3, 1921.

2 SHEETS—SHEET 1.



Inventor  
Nelson P. Bump

N. P. BUMP,  
GUN STOCK FOR RIFLES, GUNS, AND SMALL ARMS.  
APPLICATION FILED MAY 29, 1918.

1,376,917.

Patented May 3, 1921.

2 SHEETS—SHEET 2.



Inventor  
*Nelson P. Bump*

# UNITED STATES PATENT OFFICE.

NELSON P. BUMP, OF BRIDGEPORT, CONNECTICUT, ASSIGNOR TO C. C. WILLIAMS,  
ACTING CHIEF OF ORDNANCE, UNITED STATES ARMY, TRUSTEE.

## GUN-STOCK FOR RIFLES, GUNS, AND SMALL-ARMS.

1,376,917.

Specification of Letters Patent.

Patented May 3, 1921.

Application filed May 29, 1918. Serial No. 237,324.

(FILED UNDER THE ACT OF MARCH 3, 1883, 22 STAT. L. 625.)

*To all whom it may concern:*

Be it known that I, NELSON PERRY BUMP, captain, Ordnance Reserve Corps, a citizen of the United States, residing at Bridgeport, 5 county of Fairfield, and State of Connecticut, have invented a new and useful Improvement in Gun-Stocks for Rifles, Guns, and Small-Arms, of which the following is a specification.

10 The invention described herein may be used by the Government, or any of its officers or employees in prosecution of work for the Government, or by any other person in the United States, without the payment of any 15 royalty thereon.

This invention purposes to relieve the extreme emergency existing at the present time due to the limited amount of green black walnut in this country suitable for the 20 manufacture of gunstocks, by utilizing lumber of a size hitherto discarded and wasted.

To this end the invention consists in making a laminated gunstock, the plies of which are composed of pieces of lumber that are 25 thinner than those necessary in turning gunstocks of one piece.

This invention in this manner greatly increases production, by making available millions of feet of dry black walnut for the 30 manufacture of gunstocks which at the present time can not be used, as lumber only about 1" thick is necessary, in place of the 2 $\frac{1}{2}$ " lumber required for the single piece gunstocks. The lumber thus used is easier 35 to kiln dry and so an increased quantity production is attained at a decreased cost. At the same time the gunstock thus made will not warp and is stronger than those heretofore made.

40 In connection with this specification reference is had to the accompanying drawings constituting a part thereof, and in which:

Figure 1 is a side elevation, partly in section, of a gunstock constructed in accordance with this invention, showing the approximate direction of the grain in the outside plies of the completed gunstock by 45 means of arrows,

Figs. 2, 3 and 4 are plan, butt-end, and 50 fore-end views of the same respectively showing the jointed method of constructing the gunstock,

Fig. 5 is an enlarged detail showing the dovetailed joint between the plies,

55 Figs. 6 and 7 are side elevation and plan

views respectively of the built up laminated plank from which the gunstock blanks are cut out and showing the approximate direction of the grain in the outside plies and also showing the plain glued type of joint. 60

Fig. 8 is a butt-end enlarged view of the plank showing the approximate direction of the grain in the three plies,

Fig. 9 is a detailed end view of a built up 65 plank showing a slightly different method of construction, and

Fig. 10 is a detailed partial view in perspective of a similar multiply construction of the plank.

In the present war in Europe a gunstock 70 has not only been called upon to withstand the shock of recoil from heavy firing charges but also great strain in protecting the body of the soldier in close combat and in beating down the wire entanglements in advance 75 over them, and for the further use as a club in attack upon the enemy in close hand to hand fighting. The old method of constructing gunstocks consisted in turning and machining them from single pieces of hard 80 wood, the grain in the finished gunstock running generally in one direction. The rough work of present methods of fighting have found this one piece gunstock lacking in strength at the small of the stock, the 85 point B, Fig. 1. A large percentage of gunstocks break at this point in actual service necessitating the retention of a large number of spares in order to maintain one 90 rifle in service.

A gunstock constructed in accordance with this invention consists of three pieces arranged in composite form as shown in Fig. 2 in which the two outside plies are designated 1 and 2 while 3 is the center or holding ply. The center ply or tang 3 is narrower than the outside or cheek plies 1 and 2. The joint 4 between the plies may be made either plain surfaced, grooved or dovetailed as desired. In Figs. 1 to 5 inclusive 100 it is shown dovetailed while in Figs. 6, 7 and 8 it is shown plain surfaced. The plies 1 and 2 are exactly similar to each other as to form and size and are held fast to the respective sides of the center ply by means of 105 water-proof glue. Water-proof glue may also be used whenever the joints are dovetailed, or joined with a tongue and groove. In accordance with this invention the dovetail joint between the plies runs throughout 110

not only the length of the "stock" proper (from B to C in Fig. 1 of the drawings) but also throughout the length of the "butt," as shown at 4 in Figs. 2, 3 and 4. The joint 5 between the laminations is clearly shown at the point 8 broken away in Fig. 1.

In Figs. 6, 7, 8 and 10 the surface between the plies is shown plain surfaced throughout the entire length of the plank 10 the plies being held firmly together by means of water-proof glue. The outside plies in each instance, however, have the grain running approximately in the direction shown in Fig. 1, *i. e.* A B C, general 15 direction A C.

The center or tang ply in each instance is selected so that the grain will be mixed and run at different angles from the grain on the outside plies throughout the length of 20 the gunstock. The effect of this construction is to create opposite stresses in the three plies which tend to keep the gunstock absolutely straight, strengthening it greatly and making it almost impossible to split.

25 Although the three-ply method of construction is preferred this invention is not limited to such construction but any number of plies may be used in building up the composite plank as shown in Figs. 9 and 10 30 wherein six pieces are shown. The joints between the various laminations may be of any desired form as hereinbefore indicated. In these views sections corresponding to ply 1 are indicated 1<sup>1</sup> and 1<sup>2</sup> while those corresponding to ply indicated 2 in the first five views are indicated 2<sup>1</sup> and 2<sup>2</sup>, similarly the center ply is indicated by 3<sup>1</sup> and 3<sup>2</sup>.

In carrying out this invention the following method of construction is employed 40 in order to attain the desired results: The green black walnut lumber is first sawed into planks about 1" thick and subjected to steam bath until completely saturated, so as to bring out the sap. The next operation 45 is to place this steamed lumber into a kiln to dry by a slow drying process which will ultimately bring the lumber to about 5% moisture content. Slow kiln drying is necessary because it does not injure the wood as 50 does fast kiln drying.

When the lumber is removed from the drying kilns it is stored in a room of normal temperature for six days to take on as much moisture as it will naturally hold. The lumber 55 is then planed and surfaced to the desired size in a room which is of the same temperature as the room in which it has been stored. The finished lumber after this operation is then stored for at least four 60 days in a room where the laminated planks are built up and glued. This method insures a correct and even moisture content for the lumber and even temperature for the gluing process.

65 After the laminated planks are con-

structed the rough gunstock blanks are band sawed from them, the templet being laid on as indicated in phantom in Fig. 6, so that the grain in the outside plies, lie in the general direction A C Fig. 1, and then 70 the rough gunstock blanks are stored in a room of normal temperature for at least four days. The blanks are then ready for turning and machining and when this is done the stock is stored in a room of normal temperature and allowed to set.

The water-proofing solution is now applied either by immersing the gunstock in linseed oil or applying linseed oil in a vacuum which process tends to saturate the 80 gunstock completely with oil. In place of using linseed oil alone as the waterproofing agent, hot linseed oil mixed with a drier may similarly be employed. The usual bronze 85 water-proofing is then applied to the butt section of the gunstock where the oiler and thong case is inserted at 5 in Fig. 1 and also to fore-end 6 and to the balance holes 7 of the gunstock. The gunstock is now placed in a room of normal temperature for two 90 days before final assembling of the completed rifle or other small arm.

It is not absolutely essential that the grain in the center ply run at different angles to the grain of the outside plies as long as the 95 center ply has a grain that is mixed. Tests have shown that the glued joint between the plies is actually stronger than the wood itself.

Thus a gunstock made in accordance with 100 this invention is a great deal stronger than one made by the single piece method of construction, while costing decidedly less because this method makes available millions 105 of feet of black walnut which is dry and absolutely useless for the manufacture of gunstocks using the one piece method. Also the offal obtained in the manufacture of the one piece gunstocks can be utilized in the manufacture of gunstocks under this invention. Further, using thinner lumber than 110 that which is used in the manufacture of one piece gunstocks *i. e.* (2<sup>1</sup>/<sub>2</sub>"') will materially hasten the kiln drying process and therefore 115 will greatly increase the rate of production of the finished stocks.

What I claim as new and desire to secure by Letters Patent is:

1. A method of forming composite gunstocks, which consists in forming laminated 120 planks, the laminations being previously steamed to remove the sap and then slowly kiln dried, the grain in the outside laminations being selected to run in the general direction from lower point of the butt to the 125 fore-end of the stock.

2. A method of forming composite gunstocks which consists in forming laminated planks, the laminations being previously 130 steamed to remove the sap, then slowly kiln-

dried, blanking out the rough stock with the grain in the outside laminations running in the general direction from the lower point of the butt to the fore end of the stock, turning and machining the blanks and water-proofing the same to form a completed gun stock.

3. A method of forming composite gun stocks, which consists in steaming thin laminations of green lumber to remove the

sap, then slowly kiln-drying the same, assembling and gluing the laminations to form planks of the desired thickness, blanking out the rough stock with the grain in the outside laminations running in the general direction from the heel of the butt to the fore end of the stock, turning and machining the blanks and water-proofing the same to form a completed gun stock. 15

NELSON P. BUMP.